

## UNITED STATES PATENT OFFICE

2,291,066

## LUBRICANT

Stanley P. Waugh, Westfield, N. J., assignor to  
Tide Water Associated Oil Company, Bayonne,  
N. J., a corporation of Delaware

No Drawing. Application January 10, 1941,  
Serial No. 373,875

6 Claims. (Cl. 252—34)

This invention relates to lubricant compositions and methods of preparing the same. More particularly, the invention is concerned with cutting oils, and especially with soluble oils such as those used in metal working operations.

It is common practice to employ cutting oils in metal working or cutting operations and the like. In such operations it is necessary to minimize friction by the presence of a lubricating film, while at the same time avoiding excessive temperature rise at the work area by continuously supplying a coolant in liberal quantity. So-called soluble oils are now commonly used for this purpose. Soluble oils so used are essentially aqueous emulsions of mineral oil in various degrees of dilution. These compositions have the advantage of supplying both lubricant and coolant in recoverable combination permitting recirculation. In metal cutting, for example, the emulsion is applied in a continuously recirculated stream to the metal at the cutting area, the oil component forming a lubricant film between the cutting tool and the metal and the aqueous component effectively removing heat. These compositions have not been entirely satisfactory, however, because of the low strength and load-carrying capacity of the lubricant film.

Means for increasing the load-carrying capacity of the lubricant film have been devised, one such means which has met with success being the incorporation into the mineral oil aqueous composition of saponified palm oil or the saponified component derived from the fatty acid mixture obtainable from palm oil by treatment with alkaline material such as triethanolamine. Such compositions are disclosed in my U. S. Patent 2,174,907. This patented composition obviates the necessity for the former practice of melting the palm oil prior to its use in cutting operations, eliminates waste of palm oil and avoids other difficulties which had been encountered in cutting operations.

It has now been discovered, according to the present invention, that certain additive substances containing phosphorus may be incorporated into cutting oils to provide mineral oil compositions having greatly improved load-carrying capacity and other advantageous properties. Soluble oils are provided which permit cutting or other working of tougher metals in shorter periods of time with resultant more rapid operation of metal working machines and extension of the field of use of soluble oils. The invention thus presents a material advantage to the modern ma-

chine shop in meeting demands for increased production of machined metal parts.

The type or class of phosphorus compounds which according to the invention has been found particularly suitable for the stated purpose includes generally compounds or substances which may be formed by reacting phosphorus containing materials with compounds containing hydroxyl groups, such as phenols or alcohols. Phosphorus acid esters of the higher aliphatic alcohols or other phosphorus derivatives of the latter are particularly suitable, dilauryl phosphate being a representative example of such esters. Also corresponding thio phosphorus esters and derivatives are contemplated. Likewise, phosphorus derivatives of certain classes of compounds containing amino groups are effective, for example the reaction products of phosphorus acids and alkylamines, a specific embodiment being the reaction product produced by reacting phosphoric acid with triethanolamine.

One surprising fact is that the stated phosphorus compounds are materially effective in soluble oils in relatively small proportions. This fact, and the unusually high load-carrying capacity of soluble oils containing these substances, indicates that these substances do more than increase the film strength of the lubricating oil; that they also impart extreme pressure properties. As is now believed in the automotive lubrication art, the effectiveness of extreme pressure additives used in heavy duty extreme pressure gear lubricants is due to a chemical reaction involving the extreme pressure additive resulting in formation on the bearing surfaces of a high load-carrying film. Test results obtained in investigation of the soluble oils of this invention strongly indicate that the phosphorus compounds employed perform a similar function. High load-carrying properties are characteristic of soluble oils of this invention containing as little as 0.1% of the stated phosphorus compounds. The proportions may vary somewhat depending upon the other constituents used in the composition and with the type of metal working intended; and it is therefore understood that the stated proportions are not to be considered as critical or limitative.

Another distinguishing feature or property of the phosphorus compounds of the type included by this invention is their compatibility with aqueous-oil emulsions of the type herein concerned. Many substances are incapable of forming, or do not readily form, stable emulsions with water and oil, or if added to or incorporated in such

emulsions will result in instability of suspended phases and cause the emulsion to break. Obviously one of the important and essential requisites of soluble oils is that they contain no constituent tending to cause emulsion instability, and one of the objectives of the present invention is to provide stable soluble oil emulsions having markedly high load-carrying capacity. The use of phosphorus compounds of the stated type does not adversely affect the stability of soluble oil emulsions and in some cases actually results in increased stability. The invention is therefore based upon discovery of the unexpected dual function of the stated phosphorus containing additives in the composition.

As a general procedure soluble oil compositions according to the present invention are prepared by the usual method comprising bringing together suitable proportions of mineral oil and fatty acids, with heating if necessary, and a substance capable of forming with the fatty acid a soap which acts as the emulsifying agent. The method of incorporating the phosphorus compounds of the invention into the composition varies somewhat with the individual compound selected for use. Phosphorus containing compounds soluble in mineral oil, for example dilauryl phosphate, may be added to the mineral oil composition just described and the resulting product marketed as a soluble oil which before use is incorporated with water to form an emulsion. Some of the phosphorus compounds, for example the phosphoric acid-triethanolamine reaction product mentioned above, are of relatively low solubility in mineral oil but are soluble in water. These are preferably incorporated with the described composition of mineral oil and soap with addition of water. Water may be added in proportions sufficient to make a ready-to-use emulsion or in lesser quantities to form an emulsion in concentrated form which can be marketed as such and diluted with water before use. Of course the oil soluble phosphorus compounds such as dilauryl phosphate may also be incorporated with water as described and marketed as concentrated or diluted emulsion if desired.

While it is to be understood that the invention includes within its scope the employment of the stated phosphorus compounds in cutting oils or soluble oils generally, and is not limited to their use in soluble oils of particular composition, it is preferred to employ these additive agents in soluble oils containing palm oil soaps of the type set forth in my aforementioned U. S. Patent No. 2,174,907 in order that the advantageous results ensuing from said compositions may be attained. In this respect the present invention may be considered an improvement over that of my stated patent. Therefore, the following illustrative examples setting forth specific embodiments of the present invention containing palm oil products are not intended to constitute limitations as to scope of invention, but are to be considered as preferred embodiments.

#### Example I

18.5 parts by weight of phosphoric acid were added to 22.5 parts by weight of triethanolamine and the mixture was heated gently. The reaction product when dried appeared as a waxy, solid material which was readily soluble in water. This reaction product was incorporated into a soluble oil of the type set forth in my stated U. S. patent as follows.

51.1 parts by weight of a mineral red oil, from a Coastal crude, having a Saybolt viscosity of 300 seconds at 100° F., and 7.3 parts by weight of palm oil having a fatty acid content of approximately 80% by weight were mixed and the mixture heated sufficiently to dissolve the palm oil in the mineral oil. To the warm solution were slowly added 3.6 parts by weight of triethanolamine, 35.0 parts by weight of water and 3.0 parts by weight of the phosphoric acid-triethanolamine reaction product described hereinabove, with constant stirring. The resulting product, after cooling was a concentrated stable emulsion suitable for dilution with water for use in cutting or other metal working operations.

#### Example II

52.5 parts by weight of the mineral oil and 7.3 parts by weight of the palm oil described in Example I were mixed and heated in the manner described in Example I at a temperature of about 160° F. until the palm oil had all dissolved. To this solution was added 1.6 parts by weight of a commercial product consisting essentially of dilauryl phosphate and known as Du Pont "Ortholeum 162" or "G. D. 162" (obtainable from E. I. Du Pont de Nemours & Company), 3.6 parts by weight of triethanolamine and 35.0 parts by weight of water were then added with stirring to the hot solution in the manner described in Example I.

The resulting composition which when cooled was of the consistency of a paste consisted of a stable soluble oil emulsion suitable for use in cutting and other metal working operations upon dilution with suitable amounts of water.

#### Example III

Another soluble oil composition was prepared using the same starting materials and in the same manner as described in Example II except that instead of 1.6 parts by weight of the dilauryl phosphate compound, 2.7% of said compound was used. A stable concentrated emulsion suitable for dilution resulted.

The products produced as in the above examples have enduring stability of emulsion upon storage and exposure to temperature extremes.

In order to obtain an indication of the relative load-carrying capacities of the soluble oil compositions of the invention they were subjected to test on the Timkin testing machine. The Timkin machine comprises a ring of carbon steel fastened to a mandrel which is rotated and a carbon steel block having a flat surface which is placed directly beneath the ring and adapted to be pressed upwardly against the ring by a pivoted lever arm. The lubricant to be tested is made to flow continuously between the block and rotating ring, and during the test weights of successively increasing magnitude are placed upon the end of the lever arm, thus increasing the force between the ring and block. After running the machine for a given period the block is removed and the scar produced by the revolving ring on the surface of the block is measured. From this measurement and from the weight required and characteristics of the lever arm, the pressure which the lubricant was able to withstand is computed.

70 Portions of each of the concentrated emulsions prepared as in Examples I, II and III were diluted, with stirring, with ten parts of water and the resulting diluted emulsions were tested on 75 the Timkin machine in the manner described

hereinabove, the ring being revolved at 600 R. P. M., which corresponded to a speed of the rubbing surface of the ring of 300 feet per minute. With each load impressed during the runs the machine was run for a five minute interval and when such load had been reached which caused failure of the oil, as evidenced by material scoring of the block, the run was terminated.

The following table shows the pressures at failure of the soluble oils of Examples I, II and III, diluted as described, as compared with a similar soluble oil prepared from palm oil, mineral oil, triethanolamine as described in my U. S. Patent No. 2,174,907 but containing no phosphorus compound (designated in the table as "A"), and palm oil alone (designated as "B"), which compositions were also tested as set forth, on the Timkin machine.

Table

| Composition      | Load at failure<br>pounds per<br>sq. in. |
|------------------|------------------------------------------|
| Example I.....   | 20,000                                   |
| Example II.....  | 27,000                                   |
| Example III..... | 32,000 to 34,000                         |
| "A".....         | 15,000 to 17,000                         |
| "B".....         | 20,000 to 21,000                         |

These comparative results show the superior effectiveness of the soluble oils of this invention. These data are particularly significant in demonstrating the increased load-carrying capacity of the soluble oils of the invention over compositions "A" and "B," which latter compositions heretofore have been considered especially effective as regards load-carrying properties.

The examples hereinabove are not intended to constitute limitations as to the scope of the invention regarding use of any particular phosphorous compound in lubricants of the type discussed herein. Other phosphorus compounds than those shown have been tested and found ef-

fective. Among these may be mentioned tricresyl phosphate and other aromatic phosphorus containing substances. Likewise, mixtures of different phosphorus containing materials incorporated in soluble oils have been found effective. For example, incorporation of both dilauryl phosphate and the stated phosphoric acid-triethanolamine reaction product in soluble oils containing saponified palm oil such as those of my stated U. S. Patent No. 2,174,907 produces particularly effective stable emulsions for the stated purpose.

I claim:

1. Lubricating composition suitable for use in metal working operations, which comprises a stable aqueous emulsion containing mineral oil, a saponified component derived from the fatty acid mixture obtainable from palm oil, and a phosphorus-containing substance effective to increase the load-carrying capacity of the composition.
2. Lubricating composition suitable for use in metal working operations which comprises a stable aqueous emulsion containing saponified palm oil, mineral oil and a reaction product of a phosphorus acid and a hydroxy organic compound, said reaction product having high load-carrying properties.
3. Lubricating composition as in claim 2, in which the reaction product is a phosphoric acid ester.
4. Lubricating composition as in claim 2, in which the reaction product is produced by reacting phosphoric acid and an alkylolamine.
5. Lubricating composition as in claim 2, in which the reaction product is produced by reacting phosphoric acid and triethanolamine.
6. Lubricating composition comprising a stable aqueous emulsion containing mineral oil, a triethanolamine soap of palm oil fatty acids and a phosphorus compound having extreme pressure characteristics.

STANLEY P. WAUGH.